# EUROPEAN PATENT SPECIFICATION

(11) **EP 3 247 783 B1**
(45) Date of publication and mention of the grant of the patent: **23.12.2020**
(21) Application number: 16740533.1
(22) Date of filing: 15.01.2016
(51) Int. Cl.: C11D 3/37, D06M 15/53, D06M 15/643

(54) **DRYING-AID FOR LAUNDRY**
TROCKNUNGSHILFSMITTEL FÜR WÄSCHE
AUXILIAIRE DE SÉCHAGE POUR BLANCHISSERIE

(30) Priority: 19.01.2015 US 201562104929 P
(43) Date of publication of application: 29.11.2017
(73) Proprietor: Diversey, Inc., Fort Mill, SC 29708 (US)
(72) Inventor: PARTE, Anant, Charlotte, NC 28277 (US); PIJNENBURG, Niels, Johannes Maria, NL-5247 TG Rosmalen (NL); WASEKAR, Parag, Ashokrao, Maharashtra (IN); GANU, Sumedh, Sanjay, Mumbai 400074 (IN); LODAYA, Yashesh, Prafull, Mumbai 400078 (IN)
(74) Representative: Grünecker Patent- und Rechtsanwälte PartG mbB
(86) International application number: PCT/US2016/013598
(87) International publication number: WO 2016/118415

(56) References cited:
- EP-A2- 0 200 325
- WO-A1-02/31093
- WO-A1-02/31093
- WO-A1-2011/107397
- WO-A1-2014/098897
- US-B2- 8 876 982
- FENG, L ET AL.: 'Microcalorimetric Study on Interaction between PEO-PPO-PEO Triblock Copolymers and Sodium Dodecyl Trioxyethylenated Sulfonate in Aqueous Solutions.' JOURNAL OF DISPERSION SCIENCE AND TECHNOLOGY. vol. 27, no. 4, 01 January 2006, pages 555 - 559, XP055468507 DOI: 10.1080/01932690500391403

## Description

### CROSS-REFERENCE TO RELATED APPLICATION

This application claims the benefit of and priority to U.S. Provisional Patent Application No. 62/104,929, filed January 19, 2015.

### BACKGROUND

Drying operations can be one of the primary bottlenecks in an industrial laundry operation if not performed efficiently. Further, drying operations consume upwards of 65% of the total energy consumed in a laundering process.

According to the Textile Rental Service Association of America, the total in-plant energy used for laundering textiles has steadily declined from about 3100 Btu per pound of laundry in 1997 to about 2260 Btu per pound of laundry in 2009. See LaundryESP® by TRSA, http://www.trsa.org/page/energy (last visited March 1, 2013). Similarly, water usage for laundering textiles has steadily declined from about 2.31 gallons per pound of laundry in 1997 to about 1.55 gallons per pound of laundry in 2009. See LaundryESP® by TRSA, http://www.trsa.org/page/water (last visited March 1, 2013). A significant portion of these efficiency gains can be attributed to systems that provide mechanical advantages to the drying process and incorporate recycling of heat and water.

Drying of laundry is generally a two-stage process: mechanical dewatering followed by thermal drying. A textile going through this process will have some initial moisture content and will undergo mechanical dewatering for some time until an intermediate moisture content is reached. Once this occurs, the textile having an intermediate moisture content will undergo thermal drying for some time until a final moisture content is reached. In both stages, the energy consumption can be reduced by either reducing the moisture content at the beginning of the stage or improving moisture removal efficiency during the stage. However, there exist only a few means of achieving these reductions and improvements.

First, the water-removal process may be improved, such that moisture removal is more efficient regardless of the textile or water used. These improvements can be made by improving the mechanical efficiency of the process, incorporating recycling of heat and water, or simply by taking advantage of components which themselves have higher energy efficiency, such as energy efficient motors and the like. Improvements to the process are generally applicable to any type of textile, and therefore result in energy savings regardless of the textile used. Reduction in energy related to improvement in the water-removal process may translate into a reduction in cost of laundering a textile only after the cost of the equipment required for the improved process has been repaid. In other words, a significant up-front investment must be made in order to achieve the benefits of improved mechanical extraction, so the savings are delayed. Furthermore, improvements to the process require a process that is not already state-of-the-art, so they are not effective to reduce energy costs for newer laundry processes.

Second, a textile may be chemically modified so as to retain less water than it otherwise would in the absence of the chemical modification. Examples of chemically-modified textiles having improved drying properties can be found in U.S. Patent Application Pub. No. 2009/0158492. While chemically modifying textiles can lead to energy savings associated with drying processes, improvements in overall laundering efficiency must take into account the costs associated with chemically modifying existing normal textiles or replacing existing normal textiles with chemically-modified textiles. A significant up-front investment thus must be made in order to achieve the benefits associated with chemically-modified textiles, thereby delaying overall savings.

Third, a composition may be added to an aqueous bath at some point during the laundering process to modify the interaction between water and the textile, such that the textile does not retain as much water as it otherwise would if the same laundering process were performed without the composition. Reductions in energy related to adding compositions to an aqueous bath are generally applicable to any type of textile, and therefore result in energy savings regardless of the textile used or the details of the extraction and drying process. While using compositions to reduce the drying time of textiles can lead to energy savings associated with the drying process, improvements in overall laundering efficiency must take into account the costs associated with the use of the composition. However, unlike the means discussed above, the up-front cost associated with adding a composition to an aqueous bath are minimal, as one needs to only purchase as much composition as one intends to use. When reduction in energy occurs as a result of adding a composition to an aqueous bath, the reduction of cost is immediate and occurs with every load of laundry, so the savings are not delayed like the means discussed above.

In discussions of laundry efficiency, emphasis is routinely placed on the first and second means of improvement (improved mechanical extraction and chemically-modifying textiles, respectively), without mentioning the possibility of the third means, namely, adding a composition to an aqueous bath. See, e.g., "Saving Money in the Laundry Room: Conserving time, energy and dollars" by Mike Bagg, American Laundry News, October 2, 2012, http://www.americanlaundrynews.com/article/saving-money-laundry-room (last visited March 1, 2013); and "Panel of Experts: Boosting Laundry Energy Efficiency and Water Conservation," American Laundry News, April 17-18, 2012, Part 1 (http://www.americanlaundrynews.com/article/panel-experts-boosting-laundry-energy-efficiency-and-water-conservation-part-1-2) and Part 2 (http://www.americanlaundrynews.com/article/panel-experts-boosting-laundry-energy-efficiency-and-water-conservation-part-2-2) (both last visited March 1, 2013). EP 0200325 discloses a method of improving the draining of water from textiles during a laundering operation. WO 2014/098897 A1 discloses a fabric conditioner containing an amine functional silicone.

Accordingly, a need exists for a drying-aid for a laundry process that is capable of reducing the drying time of a textile at a cost low enough that the energy savings translate into cost reduction, without the up-front costs associated with the equipment required to achieve improved mechanical extraction or chemical modification of textiles.

### SUMMARY

The present invention provides a process for laundering a textile, the process comprising:
A) contacting a textile with an aqueous rinse bath;
B) separating the textile from the aqueous rinse bath; and
C) drying the textile,
wherein the aqueous rinse bath comprises from 0.05 g to 10 g of an ethylene oxide-propylene oxide-ethylene oxide (EO/PO/EO) triblock copolymer per kg of textile; from 0.01 g to 7.5 g of an aminosilicone per kg of textile; and a weight ratio of the triblock copolymer to the aminosilicone in a range of from 5:1 to 25:1.

Preferred embodiments of the invention are set forth in the subclaims.

The process of the invention is suitable for lowering a cost of laundering a textile.

Other aspects of the invention will become apparent by consideration of the detailed description and accompanying drawings.

### BRIEF DESCRIPTION OF THE DRAWINGS

Fig. 1 is a plot of the data acquired in Example 4, graphing the percent reduction in drying time versus the dosage of drying-aid composition.

### DETAILED DESCRIPTION

This disclosure is not limited in its application to the details of construction and the arrangement of components set forth in the following description. The disclosure may provide other embodiments and may be practiced or carried out in various ways. Also, it is to be understood that the phraseology and terminology used herein is for the purpose of description and should not be regarded as limiting. The use of "including," "comprising," or "having" and variations thereof herein is meant to encompass the items listed thereafter and equivalents thereof as well as additional items.

It also is understood that any numerical range recited herein includes all values from the lower value to the upper value. For example, if a concentration range is stated as 1% to 50%, it is intended that values such as 2% to 40%, 10% to 30%, or 1% to 3%, etc., are expressly enumerated in this specification. These are only examples of what is specifically intended, and all possible combinations of numerical values between and including the lowest value and the highest value enumerated are to be considered to be expressly stated in this application.

It should be understood that, as used herein, the term "about" is synonymous with the term "approximately." Illustratively, the use of the term "about" indicates that a value includes values slightly outside the cited values. Variation may be due to conditions such as experimental error, manufacturing tolerances, variations in equilibrium conditions, and the like. In some embodiments, the term "about" includes the cited value plus or minus 10%. In all cases, where the term "about" has been used to describe a value, it should be appreciated that this disclosure also supports the exact value.

This disclosure provides a process for laundering a textile, as described in detail below.

### I. Compositions

This disclosure provides a process that is suitable for reducing a drying time of a textile after immersion in an aqueous bath by adding a composition to the aqueous bath. The composition comprises an ethylene oxide-propylene oxide-ethylene oxide (EO/PO/EO) triblock copolymer and an aminosilicone. In one aspect, the composition is a stable formulation which contains an EO/PO/EO triblock copolymer and an aminosilicone.

It has been observed that adding a composition comprising either an EO/PO/EO triblock copolymer or an aminosilicone to an aqueous bath containing a textile causes an overall reduction in the drying time of the textile. Moreover, it was surprisingly discovered that compositions comprising both an EO/PO/EO triblock copolymer and an aminosilicone, when added to an aqueous bath containing a textile, reduce the drying time of the textile more so than compositions comprising either the EO/PO/EO triblock copolymer alone, or the aminosilicone alone. In other words, the EO/PO/EO triblock copolymer and aminosilicone, when provided together in a single composition appear to have a synergistic effect on the efficiency of the drying process.

The amount of EO/PO/EO triblock copolymer (by weight of the active ingredient) in the composition may be at least 5%, such as at least 10%, at least 15%, at least 20%, at least 25%, at least 30%, at least 35%, at least 40%, at least 45%, at least 50%, at least 55%, at least 60%, at least 65%, at least 70%, at least 75%, at least 80%, at least 85%, at least 90%, or at least 95%. The amount of EO/PO/EO triblock copolymer (by weight) in the composition may be at most 99%, such as at most 95%, at most 90%, at most 85%, at most 80%, at most 75%, at most 70%, at most 65%, at most 60%, at most 55%, at most 50%, at most 45%, at most 40%, at most 35%, at most 30%, at most 25%, at most 20%, at most 15%, or at most 10%. This includes embodiments where the amount of EO/PO/EO triblock copolymer (by weight) in the composition ranges from 5% to 95% including, but not limited to, amounts ranging from 10% to 90%, from 15% to 85%, from 20% to 80%, and from 25% to 75%.

The amount of aminosilicone (by weight of the active ingredient) in the composition may be at least 1%, such as at least 2%, at least 3%, at least 4%, at least 5%, at least 6%, at least 7%, at least 8%, at least 9%, at least 10%, at least 11%, at least 12%, at least 13%, at least 14%, at least 15%, at least 16%, at least 17%, at least 18%, at least 19%, at least 20%, at least 21%, at least 22%, at least 23%, or at least 24%. The amount of aminosilicone (by weight) in the composition may be at most 25%, such as at most 24%, at most 23%, at most 22%, at most 21%, at most 20%, at most 19%, at most 18%, at most 17%, at most 16%, at most 15%, at most 14%, at most 13%, at most 12%, at most 11%, at most 10%, at most 9%, at most 8%, at most 7%, at most 6%, at most 5%, at most 4%, at most 3%, or at most 2%. This includes embodiments where the amount of aminosilicone (by weight) in the composition ranges from 1% to 25% including, but not limited to, amounts ranging from 2% to 24%, from 3% to 23%, from 4% to 22%, from 5% to 21%, from 6% to 20%, from 7% to 19%, from 8% to 18%, from 9% to 17%, and from 10% to 16%.

The compositions disclosed herein comprise a ratio (by weight of the active ingredients) of EO/PO/EO triblock copolymer to aminosilicone of at least 5:1, such as at least 5.5:1, at least 6:1, at least 6.5:1, at least 7:1, at least 7.5:1, at least 8:1, at least 8.5:1, at least 9:1, at least 9.5:1, at least 10:1, at least 10.5:1, at least 11:1, at least 11.5:1, at least 12:1, at least 12.5:1, at least 13:1, at least 13.5:1, at least 14:1, at least 14.5:1, at least 15:1, at least 15.5:1, at least 16:1, at least 16.5:1, at least 17:1, at least 17.5:1, at least 18:1, at least 18.5:1, at least 19:1, at least 19.5:1, at least 20:1, at least 21:1, at least 22:1, at least 23:1, at least 24:1, or at least 25:1. The compositions disclosed herein comprise a ratio (by weight) of EO/PO/EO block copolymer to aminosilicone of at most 25:1, such as at most 24:1, at most 23:1, at most 22:1, at most 21:1, at most 20:1, at most 19.5:1, at most 19:1, at most 18.5:1, at most 18:1, at most 17.5:1, at most 17:1, at most 16.5:1, at most 16:1, at most 15.5:1, at most 15:1, at most 14.5:1, at most 14:1, at most 13.5:1, at most 13:1, at most 12.5:1, at most 12:1, at most 11.5:1, at most 11:1, at most 10.5:1, at most 10:1, at most 9.5:1, at most 9:1, at most 8.5:1, at most 8:1, at most 7.5:1, at most 7:1, at most 6.5:1, at most 6:1, at most 5.5:1, or at most 5:1. This includes embodiments where the ratio (by weight) of EO/PO/EO block copolymer to aminosilicone in the composition ranges from 5:1 to 15:1, from 5.5:1 to 14.5:1, from 6:1 to 14:1, from 6.5:1 to 13.5:1, from 7:1 to 13:1, from 7.5:1 to 12.5:1, from 8:1 to 12:1, from 8.5:1 to 11.5:1, and from 9:1 to 11:1.

In some embodiments, the composition further may comprise one or more fabric softeners. Fabric softeners may include one or more components, including at least one fabric softener active component that functions to soften textiles. Suitable fabric softeners may include, but are not limited to those disclosed in U.S. Patent Publication Nos. 2006/0089293, 2006/0264352, 2009/0203570, and 2012/0324652, and U.S. Patent Nos. 3,972,131, 4,035,307, 4,661,267, 5,002,681, 5,500,138, 5,726,144, 5,977,055, 6,492,322 , 6,583,105, 6,939,844, and 7,381,697, among others. Use of a fabric softener in compositions disclosed herein, may provide ease of use, such that a single composition can be introduced into the laundering process in the same fashion as the fabric softener is currently introduced.

In embodiments comprising a fabric softener, the compositions disclosed herein may comprise a ratio (by weight of the active ingredients) of EO/PO/EO block copolymer and aminosilicone combined to fabric softener of at least 1:10, such as at least 1:9, at least 1:8, at least 1:7, at least 1:6, at least 1:5, at least 1:4, at least 1:3, or at least 1:2. The compositions disclosed herein may comprise a ratio (by weight) of EO/PO/EO block copolymer and aminosilicone combined to fabric softener (as 100% active) of at most 1:1, such as at most 1:2, at most 1:3, at most 1:4, at most 1:5, at most 1:6, at most 1:7, at most 1:8, or at most 1:9. This includes, but is not limited to embodiments where the ratio (by weight) of EO/PO/EO block copolymer and aminosilicone combined to fabric softener (as 100% active) ranges from 1:10 to 1:1, including, but not limited to, ratios ranging from 1:8 to 1:3, and from 1:7.5 to 1:4.

In some embodiments, the compositions disclosed herein are added to an aqueous bath to yield a combined amount of EO/PO/EO block copolymer and aminosilicone in the aqueous bath of at least 0.1 g per kg of textile, such as at least 0.2 g, at least 0.3 g, at least 0.4 g, at least 0.5 g, at least 0.6 g, at least 0.7 g, at least 0.8 g, at least 0.9 g, at least 1.0 g, at least 1.1 g, at least 1.2 g, at least 1.3 g, at least 1.4 g, at least 1.5 g, at least 1.6 g, at least 1.7 g, at least 1.8 g, at least 1.9 g, at least 2.0 g, at least 2.1 g, at least 2.2 g, at least 2.3 g, at least 2.4 g, at least 2.5 g, at least 2.6 g, at least 2.7 g, at least 2.8 g, at least 2.9 g, at least 3.0 g, at least 3.1 g, at least 3.2 g, at least 3.3 g, at least 3.4 g, at least 3.5 g, at least 3.6 g, at least 3.7 g, at least 3.8 g, at least 3.9 g, at least 4.0 g, at least 4.1 g, at least 4.2 g, at least 4.3 g, at least 4.4 g, at least 4.5 g, at least 4.6 g, at least 4.7 g, at least 4.8 g, at least 4.9 g, at least 5.0 g, at least 5.5 g, at least 6.0 g, at least 6.5 g, at least 7.0 g, at least 7.5 g, at least 8.0 g, at least 8.5 g, at least 9.0 g, or at least 9.5 g per kg of textile. When added to an aqueous bath, the compositions disclosed herein may yield a combined amount of EO/PO/EO block copolymer and aminosilicone in the aqueous bath of at most 10.0 g per kg of textile, such as at most 9.5 g, at most 9.0 g, at most 8.5 g, at most 8.0 g, at most 7.5 g, at most 7.0 g, at most 6.5 g, at most 6.0 g, at most 5.5 g, at most 5.0 g, at most 4.9 g, at most 4.8 g, at most 4.7 g, at most 4.6 g, at most 4.5 g, at most 4.4 g, at most 4.3 g, at most 4.2 g, at most 4.1 g, at most 4.0 g, at most 3.9 g, at most 3.8 g, at most 3.7 g, at most 3.6 g, at most 3.5 g, at most 3.4 g, at most 3.3 g, at most 3.2 g, at most 3.1 g, at most 3.0 g, at most 2.9 g, at most 2.8 g, at most 2.7 g, at most 2.6 g, at most 2.5 g, at most 2.4 g, at most 2.3 g, at most 2.2 g, at most 2.1 g, at most 2.0 g, at most 1.9 g, at most 1.8 g, at most 1.7 g, at most 1.6 g, at most 1.5 g, at most 1.4 g, at most 1.3 g, at most 1.2 g, at most 1.1 g, at most 1.0 g, at most 0.9 g, at most 0.8 g, at most 0.7 g, at most 0.6 g, at most 0.5 g, at most 0.4 g, at most 0.3 g, or at most 0.2 g per kg of textile. This includes embodiments where adding the composition to the aqueous bath yields a combined amount of EO/PO/EO triblock copolymer and aminosilicone in the aqueous bath ranging from 0.1 g per kg of textile to 10.0 g per kg of textile, including, but not limited to, amounts ranging from 0.5 g per kg of textile to 5.0 g per kg of textile, from 0.75 g per kg of textile to 4.0 g per kg of textile, and from 1.0 g per kg of textile to 3.0 g per kg of textile.

When added to an aqueous bath, the compositions disclosed herein may yield an amount of EO/PO/EO triblock copolymer in the aqueous bath of at least 0.05 g per kg of textile, such as at least 0.1 g, at least 0.2 g, at least 0.3 g, at least 0.4 g, at least 0.5 g, at least 0.6 g, at least 0.7 g, at least 0.8 g, at least 0.9 g, at least 1.0 g, at least 1.1 g, at least 1.2 g, at least 1.3 g, at least 1.4 g, at least 1.5 g, at least 1.6 g, at least 1.7 g, at least 1.8 g, at least 1.9 g, at least 2.0 g, at least 2.1 g, at least 2.2 g, at least 2.3 g, at least 2.4 g, at least 2.5 g, at least 2.6 g, at least 2.7 g, at least 2.8 g, at least 2.9 g, at least 3.0 g, at least 3.1 g, at least 3.2 g, at least 3.3 g, at least 3.4 g, at least 3.5 g, at least 3.6 g, at least 3.7 g, at least 3.8 g, at least 3.9 g, at least 4.0 g, at least 4.1 g, at least 4.2 g, at least 4.3 g, at least 4.4 g, at least 4.5 g, at least 4.6 g, at least 4.7 g, at least 4.8 g, at least 4.9 g, at least 5.0 g, at least 5.5 g, at least 6.0 g, at least 6.5 g, at least 7.0 g, at least 7.5 g, at least 8.0 g, at least 8.5 g, at least 9.0 g, or at least 9.5 g per kg of textile. When added to an aqueous bath, the compositions disclosed herein may yield an amount of EP/PO/EO triblock copolymer in the aqueous bath of at most 9.8 g per kg of textile, such as at most 9.5 g, at most 9.0 g, at most 8.5 g, at most 8.0 g, at most 7.5 g, at most 7.0 g, at most 6.5 g, at most 6.0 g, at most 5.5 g, at most 5.0 g, at most 4.9 g, at most 4.8 g, at most 4.7 g, at most 4.6 g, at most 4.5 g, at most 4.4 g, at most 4.3 g, at most 4.2 g, at most 4.1 g, at most 4.0 g, at most 3.9 g, at most 3.8 g, at most 3.7 g, at most 3.6 g, at most 3.5 g, at most 3.4 g, at most 3.3 g, at most 3.2 g, at most 3.1 g, at most 3.0 g, at most 2.9 g, at most 2.8 g, at most 2.7 g, at most 2.6 g, at most 2.5 g, at most 2.4 g, at most 2.3 g, at most 2.2 g, at most 2.1 g, at most 2.0 g, at most 1.9 g, at most 1.8 g, at most 1.7 g, at most 1.6 g, at most 1.5 g, at most 1.4 g, at most 1.3 g, at most 1.2 g, at most 1.1 g, at most 1.0 g, at most 0.9 g, at most 0.8 g, at most 0.7 g, at most 0.6 g, at most 0.5 g, at most 0.4 g, at most 0.3 g, at most 0.2 g, or at most 0.1 g per kg of textile. This includes embodiments where adding the composition to the aqueous bath yields an amount of EO/PO/EO triblock copolymer in the aqueous bath ranging from 0.05 g per kg of textile to 9.8 g per kg of textile, including, but not limited to, amounts ranging from 0.5 g per kg of textile to 9.5 g per kg of textile, from 1.0 g per kg of textile to 9.0 g per kg of textile, and from 2.0 g per kg of textile to 8.0 g per kg of textile.

When added to an aqueous bath, the compositions disclosed herein may yield an amount of aminosilicone in the aqueous bath of at least 0.01 g per kg of textile, such as at least 0.20 g, at least 0.04 g, at least 0.06 g, at least 0.08 g, at least 0.1 g, at least 0.2 g, at least 0.3 g, at least 0.4 g, at least 0.5 g, at least 0.6 g, at least 0.7 g, at least 0.8 g, at least 0.9, at least 1.0 g, at least 1.1 g, at least 1.2 g, at least 1.3 g, at least 1.5 g, at least 1.6 g, at least 1.7 g, at least 1.8 g, at least 1.9 g, at least 2.0 g, at least 2.1 g, at least 2.2 g, at least 2.3 g, at least 2.4 g, at least 2.5 g, at least 2.6 g, at least 2.7 g, at least 2.8 g, at least 2.9 g, at least 3.0 g, at least 3.1 g, at least 3.2 g, at least 3.3 g, at least 3.4 g, at least 3.5 g, at least 3.6 g, at least 3.7 g, at least 3.8 g, at least 3.9 g, at least 4.0 g, at least 4.1 g, at least 4.2 g, at least 4.3 g, at least 4.4 g, at least 4.5 g, at least 4.6 g, at least 4.7 g, at least 4.8 g, at least 4.9 g, at least 5.0 g, at least 5.5 g, at least 6.0 g, at least 6.5 g, or at least 7.0 g per kg of textile. When added to an aqueous bath, the compositions disclosed herein may yield an amount of aminosilicone in the aqueous bath of at most 7.5 g per kg of textile, such as at most 7.0 g, at most 6.5 g, at most 6.0 g, at most 5.5 g, at most 5.0 g, at most 4.9 g, at most 4.8 g, at most 4.7 g, at most 4.6 g, at most 4.5 g, at most 4.4 g, at most 4.3 g, at most 4.2 g, at most 4.1 g, at most 4.0 g, at most 3.9 g, at most 3.8 g, at most 3.7 g, at most 3.6 g, at most 3.5 g, at most 3.4 g, at most 3.3 g, at most 3.2 g, at most 3.1 g, at most 3.0 g, at most 2.9 g, at most 2.8 g, at most 2.7 g, at most 2.6 g, at most 2.5 g, at most 2.4 g, at most 2.3 g, at most 2.2 g, at most 2.1 g, at most 2.0 g, at most 1.9 g, at most 1.8 g, at most 1.7 g, at most 1.6 g, at most 1.5 g, at most 1.4 g, at most 1.3 g, at most 1.2 g, at most 1.1 g, at most 1.0 g, at most 0.9 g, at most 0.8 g, at most 0.7 g, at most 0.6 g, at most 0.5 g, at most 0.4 g, at most 0.3 g, at most 0.2 g, at most 0.2 g, at most 0.1 g, at most 0.08 g, at most 0.06 g, at most 0.04 g, or at most 0.02 g per kg of textile. This includes embodiments where adding the composition to the aqueous bath yields an amount of aminosilicone in the aqueous bath ranging from 0.01 g per kg of textile to 7.5 g per kg of textile, including, but not limited to, amounts ranging from 0.1 g per kg of textile to 7.5 g per kg of textile, from 0.5 g per kg of textile to 7.0 g per kg of textile, from 1.0 g per kg of textile to 6.5 g per kg of textile, and from 2.0 g per kg of textile to 5.5 g per kg of textile.

When added to an aqueous bath, the compositions disclosed herein may reduce the drying time of a textile after immersion in the aqueous bath by at least 0.1% when compared to an aqueous bath wherein the EO/PO/EO block copolymer and aminosilicone are absent, such as by at least 0.5%, at least 1%, at least 2%, at least 3%, at least 4%, at least 5%, at least 6%, at least 7%, at least 8%, at least 9%, at least 10%, at least 11%, at least 12%, at least 13%, at least 14%, at least 15%, at least 16%, at least 17%, at least 18%, at least 19%, at least 20%, at least 21%, at least 22%, at least 23%, at least 24%, at least 25%, at least 26%, at least 27%, at least 28%, at least 29%, or at least 30% when compared to an aqueous bath wherein the EO/PO/EO block copolymer and aminosilicone are absent. Unless otherwise indicated, the term "drying time" means the time required to dry a textile in a tumble drying process.

When added to an aqueous bath, the compositions disclosed herein may reduce the drying time of a textile after immersion in the aqueous bath by at least 0.1% when compared to an aqueous bath wherein the EO/PO/EO block copolymer and aminosilicone are each replaced with an equal volume of fabric softener, such as by at least 0.5%, at least 1%, at least 2%, at least 3%, at least 4%, at least 5%, at least 6%, at least 7%, at least 8%, at least 9%, at least 10%, at least 11%, at least 12%, at least 13%, at least 14%, at least 15%, at least 16%, at least 17%, at least 18%, at least 19%, at least 20%, at least 21%, at least 22%, at least 23%, at least 24%, or at least 25% when compared to an aqueous bath wherein the EO/PO/EO block copolymer and aminosilicone are each replaced by an equal volume of fabric softener.

In some embodiments, the aqueous bath may be at a temperature of at least 15° C, at least 16° C, at least 17° C, at least 18° C, at least 19° C, at least 20° C, at least 21° C, at least 22° C, at least 23° C, at least 24° C, at least 25° C, at least 26° C, at least 27° C, at least 28° C, at least 29° C, at least 30° C, at least 31° C, at least 32° C, at least 33° C, at least 34° C, at least 35° C, at least 36° C, at least 37° C, at least 38° C, at least 39° C, at least 40° C, at least 41° C, at least 42° C, at least 43° C, at least 44° C, at least 45° C, at least 46° C, at least 47° C, at least 48° C, at least 49° C, at least 50° C, at least 51° C, at least 52° C, at least 53° C, at least 54° C, at least 55° C, at least 56° C, at least 57° C, at least 58° C, at least 59° C, or at least 60° C. In some embodiments, the aqueous bath may be at a temperature of at most 60° C, at most 59° C, at most 58° C, at most 57° C, at most 56° C, at most 55° C, at most 54° C, at most 53° C, at most 52° C, at most 51° C, at most 50° C, at most 49° C, at most 48° C, at most 47° C, at most 46° C, at most 45° C, at most 44° C, at most 43° C, at most 42° C, at most 41° C, at most 40° C, at most 39° C, at most 38° C, at most 37° C, at most 36° C, at most 35° C, at most 34° C, at most 33° C, at most 32° C, at most 31° C, at most 30° C, at most 29° C, at most 28° C, at most 27° C, at most 26° C, at most 25° C, at most 24° C, at most 23° C, at most 22° C, at most 21° C, at most 20° C, at most 19° C, at most 18° C, at most 17° C, at most 16° C, or at most 15° C. This includes temperatures ranging from 15° C to 60° C, including but not limited to, temperatures ranging from 20° C to 50° C, and from 25° C to 45° C. In some embodiments, the aqueous bath may be at room temperature, which means from 20° C to 25° C.

In some embodiments, the aqueous bath may have a pH of at least 3, at least 3.1 , at least 3.2, at least 3.3, at least 3.4, at least 3.5, at least 3.6, at least 3.7, at least 3.8, at least 3.9, at least 4.0, at least 4.1, at least 4.2, at least 4.3, at least 4.4, at least 4.5, at least 4.6, at least 4.7, at least 4.8, at least 4.9, at least 5.0, at least 5.1, at least 5.2, at least 5.3, at least 5.4, at least 5.5, at least 5.6, at least 5.7, at least 5.8, at least 5.9, at least 6.0, at least 6.1, at least 6.2, at least 6.3, at least 6.4, at least 6.5, at least 6.6, at least 6.7, at least 6.8, at least 6.9, at least 7.0, at least 7.1, at least 7.2, at least 7.3, at least 7.4, at least 7.5, at least 7.6, at least 7.7, at least 7.8, at least 7.9, at least 8.0, at least 8.1, at least 8.2, at least 8.3, or at least 8.4. In some embodiments, the aqueous bath may have a pH of at most 8.5, at most 8.4, at most 8.3, at most 8.2, at most 8.1, at most 8.0, at most 7.9, at most 7.8, at most 7.7, at most 7.6, at most 7.5, at most 7.4, at most 7.3, at most 7.2, at most 7.1, at most 7.0, at most 6.9, at most 6.8, at most 6.7, at most 6.6, at most 6.5, at most 6.4, at most 6.3, at most 6.2, at most 6.1, at most 6.0, at most 5.9, at most 5.8, at most 5.7, at most 5.6, at most 5.5, at most 5.4, at most 5.3, at most 5.2, at most 5.1, at most 5.0, at most 4.9, at most 4.8, at most 4.7, at most 4.6, at most 4.5, at most 4.4, at most 4.3, at most 4.2, at most 4.1, at most 4.0, at most 3.9, at most 3.8, at most 3.7, at most 3.6, at most 3.5, at most 3.4, at most 3.3, at most 3.2, or at most 3.1. This includes embodiments where the pH values ranging from 3 to 8.5, including, but not limited to, values ranging from 3.5 to 8, and from 4.0 to 7.5.

### A. EO/PO/EO Triblock Copolymer

The compositions disclosed herein comprise an EO/PO/EO triblock copolymer.

In some embodiments, the EO/PO/EO triblock copolymer may have a molar mass of at least 500 g/mol, at least 600 g/mol, at least 700 g/mol, at least 800 g/mol, at least 900 g/mol, at least 1000 g/mol, at least 1100 g/mol, at least 1200 g/mol, at least 1300 g/mol, at least 1400 g/mol, at least 1500 g/mol, at least 1600 g/mol, at least 1700 g/mol, at least 1800 g/mol, at least 1900 g/mol, at least 2000 g/mol, at least 2250 g/mol, at least 2500 g/mol, at least 2750 g/mol, at least 3000 g/mol, at least 3250 g/mol, at least 3500 g/mol, at least 3750 g/mol, at least 4000 g/mol, at least 4250 g/mol, at least 4500 g/mol, or at least 4750 g/mol. In some embodiments, the EO/PO/EO triblock copolymer may have a molar mass of at most 5000 g/mol, at most 4750 g/mol, at most 4500 g/mol, at most 4250 g/mol, at most 4000 g/mol, at most 3750 g/mol, at most 3500 g/mol, at most 3250 g/mol, at most 3000 g/mol, at most 2500 g/mol, at most 2000 g/mol, at most 1500 g/mol, or at most 1000 g/mol. This includes embodiments, where the EO/PO/EO triblock copolymer has a molar mass ranging from 500 g/mol to 5000 g/mol, including, but not limited to, molar mass ranging from 1000 g/mol to 4500 g/mol, and from 1500 g/mol to 4000 g/mol.

In some embodiments, the EO/PO/EO triblock copolymer comprises a PO block that may have a molar mass of at least 450 g/mol, at least 500 g/mol, at least 600 g/mol, at least 700 g/mol, at least 800 g/mol, at least 900 g/mol, at least 1000 g/mol, at least 1100 g/mol, at least 1200 g/mol, at least 1300 g/mol, at least 1400 g/mol, at least 1500 g/mol, at least 1600 g/mol, at least 1700 g/mol, at least 1800 g/mol, at least 1900 g/mol, at least 2000 g/mol, at least 2250 g/mol, at least 2500 g/mol, at least 2750 g/mol, at least 3000 g/mol, at least 3250 g/mol, at least 3500 g/mol, at least 3750 g/mol, at least 4000 g/mol, or at least 4250 g/mol. In some embodiments, the EO/PO/EO triblock copolymer comprises a PO block that may have a molar mass of at most 4500 g/mol, at most 4250 g/mol, at most 4000 g/mol, at most 3750 g/mol, at most 3500 g/mol, at most 3250 g/mol, at most 3000 g/mol, at most 2500 g/mol, at most 2000 g/mol, at most 1500 g/mol, at most 1000 g/mol, at most 750 g/mol, or at most 500 g/mol. This includes embodiments where the EO/PO/EO triblock copolymer comprises a PO block having a molar mass ranging from 450 g/mol to 4500 g/mol, including, but not limited to, molar masses ranging from 500 g/mol to 4250 g/mol, and from 1000 g/mol to 4000 g/mol.

In some embodiments, the EO/PO/EO triblock copolymer may comprise at least 1% by weight EO, at least 2%, at least 3%, at least 4%, at least 5%, at least 6%, at least 7%, at least 8%, at least 9%, at least 10%, at least 11%, at least 12%, at least 13%, at least 14%, at least 15%, at least 16%, at least 17%, at least 18%, at least 19%, at least 20%, at least 21%, at least 22%, at least 23%, at least 24%, at least 25%, at least 30%, at least 35%, at least 40%, at least 45%, at least 50%, at least 55%, at least 60%, at least 65%, at least 70%, at least 75%, at least 80%, or at least 85% by weight EO. In some embodiments, the EO/PO/EO triblock copolymer may comprise at most 90% by weight EO, at most 85%, at most 80%, at most 75%, at most 70%, at most 65%, at most 60%, at most 55%, at most 50%, at most 45%, at most 40%, at most 35%, at most 30%, at most 25%, at most 24%, at most 23%, at most 22%, at most 21%, at most 20%, at most 19%, at most 18%, at most 17%, at most 16%, at most 15%, at most 14%, at most 13%, at most 12%, at most 11%, at most 10%, at most 9%, at most 8%, at most 7%, at most 6%, at most 5%, at most 4%, at most 3, or at most 2% by weight EO. This includes embodiments where the EO/PO/EO triblock copolymer comprises an amount of EO by weight ranging from 1% to 90%, including, but not limited to, amounts ranging from 5% to 85%, from 10% to 80%, from 15% to 75%, and from 20% to 70. Preferably, the EO/PO/EO triblock copolymer comprises an amount of EO by weight ranging from 1% to 25%, such as from 2% to 20%, and from 5% to 15%.

Commercially available EO/PO/EO triblock copolymers suitable for use in this invention include Pluronic® PE series (available from BASF) and the Tergitol™ series (available from Dow Chemical).

### B. Aminosilicone

In some embodiments, the aminosilicone may comprise cationic polydialkylsiloxanes with amino functional groups. The alkyl groups in the polydialkylsiloxanes include C1-C10 alkyl groups, such as methyl, ethyl, propyl, isopropyl, n-butyl, isobutyl, pentyl, hexyl, heptyl, octyl, nonyl, and decyl groups. For example, the aminosilicone of the present disclosure can comprise polydimethyl-, polydiethyl-, polydipropyl- or polydibutylsiloxanes with amino functional groups. Preferably, the aminosilicone comprises polydimethylsiloxane with amino functional groups.

Commercially available aminosilicones suitable for use in this invention may include Wacker® aminosilicones.

### C. Fabric Softener

In some embodiments, the fabric softener may comprise any suitable fabric softener known to one of skill in the art. Suitable softener may contain 5-20% by weight cationic surfactant.

Commercially available fabric softeners suitable for use in this invention may include Clax Xtra Soft (available from Diversey, Sturtevant, WI).

### D. Additional Components

In some embodiments, the drying aid composition may contain one or more additional components. For example, the additional components can be included to achieve a stable formulation. A stable formulation means a formulation in which no precipitation or phase separation occur during a prolonged storage period (for example, at least 3 months) at various temperatures (such as -10 °C, 5 °C, 20 °C, 40 °C, or 50 °C). The additional components may include, but are not limited to, nonionic surfactant, emulsifier, polyethylene glycol (PEG), alcoholic solvent, thickener, and preservative. Suitable nonionic surfactants may include, but are not limited to, alkylpolyethylene glycol ethers and PO/EO block polymer. Examples of commercial nonionic surfactants include Lutensol AT80 (BASF), an alkylpolyethylene glycol ethers made from a linear, saturated C16-C18 fatty alcohol and Pluronic PE10500 (BASF), and a PO/EO block polymer. Suitable emulsifiers include, but are not limited to, alcohol ethoxylates, such as Emulan HE50 (BASF). Suitable polyethylene glycols may include, but are not limited to, PEG 200 and PEG 400. Suitable alcoholic solvents may include, but are not limited to, isopropyl alcohol (IPA) and ethanol. Suitable thickeners may include, but are not limited to, cellulosic thickeners, such as carboxymethylcellulose, hydroxypropyl methylcellulose, and hydroxyethyl cellulose. Examples of commercial cellulosic thickeners include FinnFix LC (CP Kelco). Suitable preservative may include, but are not limited to, 1,2-benzisothiazolin-3-one, such as the commercial product Proxel GXL (Lonza).

### II. Uses of Compositions

The compositions described herein may be used to lower a cost of drying a textile.

In some embodiments, the cost may be reduced by at least 1%, at least 2%, at least 3%, at least 4%, at least 5%, at least 6%, at least 7%, at least 8%, at least 9%, at least 10%, at least 11%, at least 12%, at least 13%, at least 14%, at least 15%, at least 16%, at least 17%, at least 18%, at least 19%, at least 20%, at least 21%, at least 22%, at least 23%, at least 24%, or at least 25%.

In some embodiments, the cost may be reduced by reducing an energy required for drying. In some embodiments, the cost may be reduced by reducing an energy required for heating a rinse bath.

In some embodiments, the energy required for drying includes steam energy, electrical energy, and/or gas energy.

### III. Methods of Lowering a Cost of Drying a Textile

Compositions described herein are employed in the process according to the invention, said process being suitable for lowering a cost of drying a textile.

One of the principle advantages of the compositions described herein is their ability to be easily incorporated into a laundering process in order to provide cost savings. A further advantage is that the lowered cost achieved by the compositions described herein is cumulative with lowered cost achieved by improved mechanical extraction or improved energy efficiency of machinery. By providing a composition that can be incorporated into existing laundering processes, the advantages can be achieved regardless of how state-of-the-art a facility may or may not be.

In principle, the methods described herein can be applied to any method of laundering a textile that involves a rinse and dry step. In preferred embodiments, the methods described herein are applied to industrial laundering processes involving a rinse step, an extraction step, and tumble drying.

### IV. Processes for Drying a Textile

Compositions described herein are employed in a process according to the invention for laundering a textile. This process is cost effective for at least the reasons stated above with respect to the compositions, their use and the methods of lowering a cost of drying a textile described herein.

In preferred embodiments, separating the textile from the aqueous bath may comprise an extraction step.

In preferred embodiments, drying the textile may comprise tumble drying.

### EXAMPLES

Exemplary embodiments of the present invention are provided in the following examples. The following examples are presented to illustrate the present invention and to assist one of ordinary skill in making and using the same. The examples are not intended in any way to otherwise limit the scope of the invention.

Use of the word linen in the Examples is intended to be illustrative of the type of textile being laundered, and not limiting the application of the compositions described herein to a particular type of textile.

As one of skill in the art would find apparent, many factors are relevant in determining the drying time, such as the external temperature and humidity conditions, fluctuations in source water temperatures, and the like. Typically, the drying tests of the present disclosure are conducted on the same day to maintain consistent conditions between the tests.

"Clax XtraSoft" or "XtraSoft" refers to Clax XtraSoft fabric softener, available commercially from Sealed Air, Duncan, SC. "Clax Soft Conc," "Soft Conc," or "SoftConc" refers to Clax Soft Conc concentrated fabric softener, available commercially from Sealed Air, Duncan, SC.

"Pluronic PE6100," "PE6100," or "PE61" refers to Pluronic® PE 6100 (available commercially from BASF Corporation, Florham Park, NJ), which is a low-foaming non-ionic surfactant. PE6100 is a block copolymer having a molar mass of about 1750 g/mol, about 10% EO in molecule, and a density of approximately 1.02 g/mL at 23° C.

"Wacker FC204" or "FC204" refers to Wacker® FC 204 (available commercially from Wacker Chemie AG, Munich, Germany), a composition containing a self-dispersing aminofunctional silicone fluid, having approximately 20% aminosilicone, and a density of approximately 1 g/mL at 20° C. "Wacker 2036M6" or "2036M6" refers to Wacker® 2036M6 (Wacker Chemie AG, Munich, Germany), a composition containing a self-dispersing aminofunctional silicone fluid, having approximately 15% aminosilicone, and a density of approximately 1 g/mL at 20° C.

"Tergitol L-61" or "L-61" refers to Tergitol™ L-61 (Dow Chemical Company, Midland, MI) nonionic surfactant, a polyether polyol. Tergitol L-61 has a density at 25° C of about 1.015 g/mL.

### Example 1. Reduced Drying Time.

About 10 kg of standard 630 GSM 100% cotton terry towels were run through a rinse cycle in an 11 kg Unimac® washer-extractor and tumble dried in an electrically heated 10 kg Primus tumble dryer. Compositions were evaluated by determining the percent water retention in the towels after final extraction and/or drying time in the tumble dryer. The percent water retention is calculated by the following equation: $% W = \frac{{w}_{w} - {w}_{i}}{{w}_{i}} \times 100$ wherein %*W* is the percent water retention, *w_{w}* is the weight of the wet towels after final spinning, hydro-extraction or drying time in the tumble dryer, and *wᵢ* is the initial weight of the dry towels kept in a conditioning room at 20° C and 55-60% relative humidity for 24 hours.

A rinse cycle and tumble drying were performed on the towels with no additive and with 8 ml of Clax XtraSoft per kg of towel (∼80 ml of Clax XtraSoft). These two experiments were performed on the same day. The results with no additive yielded a 61.25% water retention after the final spin extraction and 65 minutes of tumble drying were required to achieve 0% water retention. The results with 8 mL of Clax XtraSoft per kg of towel as additive yielded a 57.20% water retention after the final spin extraction and 61 minutes of tumble drying were required to achieve 0% water retention. This establishes that adding a fabric softener to a rinse cycle can reduce drying time. From this point forward, the reduction in drying time that was achieved by adding a fabric softener was considered to be the reference for comparison.

The compositions of Table 1 were introduced as an additive to the rinse cycle and tumble drying described in this Example, and the experiments were performed on the same day. The percent water retention after extraction, the tumble drying time required to achieve 0% water retention and corresponding percent reduction in drying time when compared with the control are also reported in Table 1.

**Table 1**

| Composition | Components (in mL per kg of textile) | | | %*W* After Extraction | Tumble Drying Time (min) | Reduction in Drying Time |
|---|---|---|---|---|---|---|
| | SoftConc | FC204 | PE6100 | | | |
| Control 1 | 3 | 0 | 0 | 65.77 | 55 | n/a |
| Comparative Example 1A | 3 | 1 | 0 | 63.64 | 52 | 6% |
| Comparative Example 1B | 3 | 2 | 0 | 65.00 | 52 | 6% |
| Comparative Example 1C | 3 | 0 | 1 | 66.29 | 56 | -2% |
| Comparative Example ID | 3 | 0 | 2 | 64.08 | 54 | 2% |
| Example 1 | 3 | 1 | 1 | 62.44 | 50 | 10% |

The data show that addition of 2 mL per kg of FC204 provides modest reduction in drying time and addition of 2 mL per kg of PE6100 provides somewhat less reduction in drying time, if any. However, when they are used together, addition of 1 mL per kg of FC204 and 1 mL per kg of PE6100 provides reduction in drying time that exceeds the reduction achieved by either component used alone.

### Example 2. Industrial Scale Reduced Drying Time.

About 92 kg of bath linen containing bath towels, hand towels, face towels, bath mats and bath robes was run through a wash and rinse cycle in a Milnor® 42022 WP2 divided-cylinder washer-extractor, with max speed of 735 rpm and hydro-extraction at 300 G-force. After extraction, about 46 kg of bath linen was loaded into a steam-heated Tumble Dryer ADC 120 (American Dryer Corp., Fall River, MA) with 54.43 kg capacity, 204.12 kg/hour steam consumption and air flow of 55.22 cmm.

The compositions of Table 2 were introduced as an additive to the rinse cycle and tumble drying described in this Example, and the experiments were performed on the same day. The tumble drying time required to achieve 0% water retention and corresponding percent reduction in drying time when compared with the control are also reported in Table 2. The experiment was repeated 8 times for the control composition and at least 2 times for the other compositions, and the results were averaged.

**Table 2**

| Composition | Components (in mL per kg of textile) | | | Tumble Drying Time (min) | Reduction in Drying Time |
|---|---|---|---|---|---|
| | SoftConc | FC204 | PE6100 | | |
| Control 2 | 5 | 0 | 0 | 48.5 | n/a |
| Comparative Example 2A | 8 | 0 | 0 | 47 | 3.09% |
| Comparative Example 2B | 5 | 2 | 0 | 42 | 13.40% |
| Comparative Example 2C | 5 | 0 | 2 | 40 | 17.53% |
| Example 2A | 5 | 1 | 1 | 38 | 21.65% |
| Example 2B | 5 | 1 | 2 | 36 | 25.77% |

The data show that addition of 2 mL per kg of FC204 and 2 mL per kg of PE6100 each provide modest reduction in drying time. However, when they are used together, addition of 1 mL per kg of FC204 and 1 or 2 mL per kg of PE6100 provides reduction in drying time that far exceeds the reduction achieved by either component used alone.

In a separate experiment, similar compositions were run through the same wash, rinse and dry cycle as described above, with the temperature of the rinse bath raised from 25° C to 45° C. These experiments were performed on the same day. The results are shown in Table 3.

**Table 3**

| Composition | Tumble Drying Time for Rinse at 25° C (min) | Tumble Drying Time for Rinse at 45° C (min) | Reduction in Drying Time |
|---|---|---|---|
| Control 2 | 48 | 42 | 12.50% |
| Comparative Example 2B | 42 | 36 | 14.29% |
| Comparative Example 2C | 40 | 35 | 12.50% |
| Example 2A | 38 | 34 | 10.53% |
| Example 2B | 36 | 34 | 5.56% |

### Example 3. Comparing Active Ingredients.

About 52 kg of bath linen containing bath towels, hand towels, face towels, bath mats and bath robes was run through a wash and rinse cycle in a Milnor® 42026 XJ7 one-cylinder washer-extractor, with a max speed of 709 rpm and hydro-extraction at 285 G-force. After extraction, about 52 kg of bath linen was loaded into a steam-heated Tumble Dryer ADC 170 (American Dryer Corp., Fall River, MA) with 54.43 kg capacity, 210.92 kg/hour steam consumption and air flow of 124.59 cmm.

The compositions of Table 4 were introduced as an additive to the rinse cycle and tumble drying described in this Example, and the experiments were performed on the same day. The tumble drying time required to achieve 0% water retention and corresponding percent reduction in drying time when compared with the control are also reported in Table 4. The experiment was repeated eight times for the control composition and at least three times for the other compositions, and the results were averaged.

**Table 4**

| Composition | Components (in mL per kg of textile) | | | | | Drying time (min) | Reduction in Drying Time |
|---|---|---|---|---|---|---|---|
| | XtraSoft | FC204 | 2036M6 | PE61 | L-61 | | |
| Control | 9.5 | 0 | 0 | 0 | 0 | 52.5 | n/a |
| Example 3A | 9.5 | 0.5 | 0 | 1.5 | 0 | 43.5 | 17.14% |
| Example 3B | 9.5 | 1.0 | 0 | 1.0 | 0 | 45.5 | 13.33% |
| Example 3C | 9.5 | 0.25 | 0 | 1.0 | 0 | 46.5 | 11.43% |
| Example 3D | 9.5 | 0 | 1.0 | 1.0 | 0 | 43.5 | 17.14% |
| Example 3E | 9.5 | 0 | 0.5 | 0 | 1.5 | 42.5 | 19.05% |

The data indicate that there may be an advantage to using more EO/PO/EO triblock copolymer than aminosilicone.

### Example 4. Dosage of Drying Aid.

The drying aid compositions of Example 4 contained a 3:1 ratio of Pluronic 6100 to Wacker 2036M6. Following the procedure of Example 3, the effect of varying the dosage of the drying aid composition was studied by adding 9.5 mL of XtraSoft per kg of linen and a dosage of the drying aid composition containing the 3:1 ratio of active ingredients as indicated in Table 5. The tumble drying time required to achieve 0% water retention was reduced when compared with the 0 mL/kg dosage. The data of Table 5 are graphed in Fig. 1.

**Table 5**

| Dosage (mL/kg) | Drying Time (min) | Reduction in Drying Time (min) |
|---|---|---|
| 0.0 | 61 | n/a |
| 1.0 | 57 | 6.56 |
| 1.5 | 54 | 11.48 |
| 2.0 | 52 | 14.75 |
| 2.5 | 51 | 16.39 |

### Example 5. Drying Aid Compositions

Several drying aid compositions were prepared and their effect in reducing drying time evaluated according to the process described in the above Examples. As shown in Table 6 (all components are expressed in weight %), these compositions contained different amounts of Pluronic PE6100 (100% EO/PO/EO block polymer) and Wacker FC204 (20% aminosilicone). The combined amount of Pluronic PE6100 and Wacker FC204 were maintained at 75% by weight of the tested compositions. Additional components were used to achieve a stabilized composition, including Lutensol AT80 (BASF), an alkylpolyethylene glycol ethers made from a linear, saturated C16-C18 fatty alcohol; Emulan HE50 (BASF), an alcohol ethoxylate; Pluronic PE10500 (BASF), a PO/EO block polymer; poly(ethylene glycol), including PEG 200 and PEG 400; isopropyl alcohol (IPA); carboxymethylcellulose, such as FinnFix LC (CP Kelco); sodium chloride; Proxel GXL (Lonza), an aqueous solution of 1,2-benzisothiazolin-3-one and dipropylene glycol; and the balance of water.

**Table 6**

| **Raw material** | **Composition 1** | **Composition 2** | **Composition 3** | **Composition 4** | **Composition 5** | **Composition 6** |
|---|---|---|---|---|---|---|
| Pluronic PE6100 (BASF) | 50 | 53.72 | 68 | 7 | 75 | 0 |
| Wacker FC204 (Wacker) | 25 | 25 | 7 | 68 | 0 | 75 |
| Lutensol AT80 (BASF) | 5 | 0 | 0.05 | 10 | 5 | 5 |
| Emulan HE50 (BASF) | 0 | 0 | 18.5 | 10 | 0 | 0 |
| Pluronic PE10500 (BASF) | 0 | 3 | 0 | 0 | 0 | 0 |
| PEG200 | 7.9 | 9 | 6.37 | 4.92 | 7.9 | 7.9 |
| PEG400 | 0 | 9 | 0 | 0 | 0 | 0 |
| Water | 5 | 0 | 0 | 0 | 5 | 5 |
| IPA | 5 | 0 | 0 | 0 | 5 | 5 |
| Finnfix LC (CP Kelco) | 0 | 0.2 | 0 | 0 | 0 | 0 |
| Sodium Chloride | 2 | 0 | 0 | 0 | 2 | 2 |
| Proxel GXL (Lonza) | 0.1 | 0.08 | 0.08 | 0.08 | 0.1 | 0.1 |
| Total | 100 | 100 | 100 | 100 | 100 | 100 |
| Reduction in drying time % | 10.9 | 14.6 | 3.9 | 6.1 | 4.2 | 7.7 |
| Standard deviation % | 1.2 | 2.7 | 1.5 | 2.4 | 1.7 | 0.2 |

The data in Table 6 shows that the synergistic effect of the combination of EO/PO/EO block polymer (Pluronic PE6100, 100% active) and aminosilicone (Wacker FC204, 20% active) in reducing drying time of the textile extends to a range of EO/PO/EO block polymer to aminosilicone weight ratios, for example, from about 49:1 (composition 3) to about 0.5:1 (composition 4). Compositions 3 and 4 are reference examples that are not embraced by the claims.

## Claims

1. A process for laundering a textile, the process comprising:
A) contacting a textile with an aqueous rinse bath;
B) separating the textile from the aqueous rinse bath; and
C) drying the textile,
wherein the aqueous rinse bath comprises from 0.05 g to 10 g of an ethylene oxide-propylene oxide-ethylene oxide (EO/PO/EO) triblock copolymer per kg of textile; from 0.01 g to 7.5 g of an aminosilicone per kg of textile; and a weight ratio of the triblock copolymer to the aminosilicone in a range of from 5:1 to 25:1.

2. The process of claim 1, wherein the EO/PO/EO triblock copolymer has a molar mass of from 500 g/mol to 5000 g/mol.

3. The process of claim 1 or 2, wherein the EO/PO/EO triblock copolymer comprises a PO block having a molar mass of from 450 g/mol to 4500 g/mol.

4. The process of any one of claims 1 to 3, wherein the EO/PO/EO triblock copolymer comprises from 1 % by weight to 25% by weight EO.

5. The process of any one of claims 1 to 4, wherein the aminosilicone comprises a polydimethylsiloxane with amino functional groups.

6. The process of any one of claims 1 to 5, wherein separating the textile from the aqueous rinse bath comprises an extraction step.

7. The process of any one of claims 1 to 6, wherein drying the textile comprises tumble drying.

8. The process of any one of claims 1-7, wherein the aqueous rinse bath is at a temperature from 20 °C to 25 °C.

9. The process of any one of claims 1-7, wherein the aqueous rinse bath is at a temperature from 15 °C to 60 °C.

10. The process of any one of claims 1-9, wherein the aqueous rinse bath has a pH from 3 to 8.5.

## Patentansprüche

1. Verfahren zum Waschen eines Textils, wobei das Verfahren umfasst:
A) Inkontaktbringen eines Textils mit einem wässrigen Spülbad;
B) Trennen des Textils von dem wässrigen Spülbad; und
C) Trocknen des Textils,
wobei das wässrige Spülbad 0,05 g bis 10 g eines Ethylenoxid-Propylenoxid-Ethylenoxid (EO/PO/EO)-Triblockcopolymers pro kg Textil; 0,01 g bis 7,5 g eines Aminosilicons pro kg Textil; und ein Gewichtsverhältnis des Triblockcopolymers zu dem Aminosilicon in einem Bereich von 5:1 bis 25:1 umfasst.

2. Verfahren nach Anspruch 1, wobei das EO/PO/EO-Triblockcopolymer eine Molmasse von 500 g/mol bis 5000 g/mol aufweist.

3. Verfahren nach Anspruch 1 oder 2, wobei das EO/PO/EO-Triblockcopolymer einen PO-Block mit einer Molmasse von 450 g/mol bis 4500 g/mol umfasst.

4. Verfahren nach einem der Ansprüche 1 bis 3, wobei das EO/PO/EO-Triblockcopolymer 1 Gew.-% bis 25 Gew.-% EO umfasst.

5. Verfahren nach einem der Ansprüche 1 bis 4, wobei das Aminosilicon ein Polydimethylsiloxan mit funktionellen Aminogruppen umfasst.

6. Verfahren nach einem der Ansprüche 1 bis 5, wobei das Abtrennen des Textils aus dem wässrigen Spülbad einen Extraktionsschritt umfasst.

7. Verfahren nach einem der Ansprüche 1 bis 6, wobei das Trocknen des Textils eine Wäschetrocknung umfasst.

8. Verfahren nach einem der Ansprüche 1 bis 7, wobei das wässrige Spülbad eine Temperatur von 20 °C bis 25 °C aufweist.

9. Verfahren nach einem der Ansprüche 1 bis 7, wobei das wässrige Spülbad eine Temperatur von 15 °C bis 60 °C aufweist.

10. Verfahren nach einem der Ansprüche 1-9, wobei das wässrige Spülbad einen pH-Wert von 3 bis 8,5 aufweist.

## Revendications

1. Procédé de blanchissage d'un textile, le procédé comprenant :
A) la mise en contact d'un textile avec un bain de rinçage aqueux ;
B) la séparation du textile du bain de rinçage aqueux ; et
C) le séchage du textile,
le bain de rinçage aqueux comprenant de 0,05 g à 10 g d'un copolymère tribloc oxyde d'éthylène-oxyde de propylène-oxyde d'éthylène (EP/PO/EO) par kg de textile ; de 0,01 g à 7,5 g d'une aminosilicone par kg de textile ; et un rapport massique du copolymère tribloc à l'aminosilicone étant dans une plage de 5:1 à 25:1.

2. Procédé selon la revendication 1, dans lequel le copolymère tribloc EO/PO/EO a une masse molaire de 500 g/mol à 5000 g/mol.

3. Procédé selon la revendication 1 ou 2, dans lequel le copolymère tribloc EO/PO/EO comprend un bloc PO ayant une masse molaire de 450 g/mol à 4500 g/mol.

4. Procédé selon l'une quelconque des revendications 1 à 3, dans lequel le copolymère tribloc EO/PO/EO comprend de 1 % en poids à 25 % en poids d'EO.

5. Procédé selon l'une quelconque des revendications 1 à 4, dans lequel l'aminosilicone comprend un polydiméthylsiloxane avec des groupes fonctionnels amino.

6. Procédé selon l'une quelconque des revendications 1 à 5, dans lequel la séparation du textile du bain de rinçage aqueux comprend une étape d'extraction.

7. Procédé selon l'une quelconque des revendications 1 à 6, dans lequel le séchage du textile comprend un séchage dans un séchoir à tambour.

8. Procédé selon l'une quelconque des revendications 1 à 7, dans lequel le bain de rinçage aqueux est à une température de 20 °C à 25 °C.

9. Procédé selon l'une quelconque des revendications 1 à 7, dans lequel le bain de rinçage aqueux est à une température de 15 °C à 60 °C.

10. Procédé selon l'une quelconque des revendications 1 à 9, dans lequel le bain de rinçage aqueux a un pH de 3 à 8,5.
